



US009177687B2

(12) **United States Patent**  
Yoshida et al.

(10) **Patent No.:** US 9,177,687 B2  
(45) **Date of Patent:** Nov. 3, 2015

(54) **COATING AND ELECTRONIC COMPONENT**

(71) **Applicant:** TDK CORPORATION, Tokyo (JP)

(72) **Inventors:** Kenichi Yoshida, Tokyo (JP); Yuhei Horikawa, Tokyo (JP); Makoto Oriksa, Tokyo (JP); Hideyuki Seike, Tokyo (JP)

(73) **Assignee:** TDK CORPORATION, Tokyo (JP)

(\*) **Notice:** Subject to any disclaimer, the term of this patent is extended or adjusted under 35 U.S.C. 154(b) by 0 days.

(21) **Appl. No.:** 13/677,509

(22) **Filed:** Nov. 15, 2012

(65) **Prior Publication Data**

US 2013/0130059 A1 May 23, 2013

(30) **Foreign Application Priority Data**

Nov. 17, 2011 (JP) ..... 2011-251349  
Nov. 14, 2012 (JP) ..... 2012-250612

(51) **Int. Cl.**

B32B 15/01 (2006.01)  
H01B 1/02 (2006.01)  
C22C 5/04 (2006.01)  
C23C 18/16 (2006.01)  
C23C 18/00 (2006.01)  
C25D 3/00 (2006.01)  
C25D 5/00 (2006.01)  
C23C 18/34 (2006.01)  
C23C 18/44 (2006.01)  
C23C 18/54 (2006.01)

(52) **U.S. Cl.**

CPC H01B 1/026 (2013.01); C22C 5/04 (2013.01);  
C23C 18/1651 (2013.01); H01B 1/02  
(2013.01); C23C 18/34 (2013.01); C23C 18/44

(2013.01); C23C 18/54 (2013.01); Y10T 428/12701 (2015.01); Y10T 428/12722 (2015.01); Y10T 428/12778 (2015.01); Y10T 428/12861 (2015.01); Y10T 428/12889 (2015.01); Y10T 428/12903 (2015.01)

(58) **Field of Classification Search**

USPC ..... 428/670  
See application file for complete search history.

(56) **References Cited**

U.S. PATENT DOCUMENTS

2007/0104929 A1\* 5/2007 Yim et al. ..... 428/209  
2009/0283884 A1\* 11/2009 Kang et al. ..... 257/676  
2010/0071940 A1\* 3/2010 Ejiri et al. ..... 174/257  
2011/0031449 A1\* 2/2011 Enomoto et al. ..... 252/513  
2011/0234215 A1\* 9/2011 Ausserlechner ..... 324/244  
2012/0018191 A1\* 1/2012 Yoshida et al. ..... 174/126.2  
2012/0118610 A1\* 5/2012 Terashima et al. ..... 174/126.2

FOREIGN PATENT DOCUMENTS

JP H07-326701 \* 5/1994 ..... C25D 5/12  
JP A-2010-037603 2/2010 .....  
WO WO 2009/099067 \* 8/2009 ..... C23C 18/44  
WO WO2011/013527 \* 2/2011 ..... C22C 5/02

\* cited by examiner

*Primary Examiner* — Humera Sheikh

*Assistant Examiner* — Lucas Wang

(74) **Attorney, Agent, or Firm:** Oliff PLC

(57) **ABSTRACT**

A coating for a conductor, the coating having a layered structure of a palladium layer. The palladium layer has a crystal plane whose orientation rate is 65% or more, which means 65% or more of the crystal planes of the palladium layer are aligned to this crystal plane. Preferably the crystal plane whose orientation rate is 65% or more in the coating is the (111) plane or (200) plane.

17 Claims, 6 Drawing Sheets



*Fig.1*

*Fig.2*

*Fig.3*

*Fig.4*

*Fig.5*

*Fig.6*

## COATING AND ELECTRONIC COMPONENT

## TECHNICAL FIELD

Some aspects of the present invention relate to a coating provided to a conductor and an electronic component including a signal transfer unit having a conductor coated with the coating.

## BACKGROUND

Electronic components include signal transfer units for sending and receiving signals to and from external apparatuses. These signal transfer units for sending and receiving electrical signals to and from external apparatuses need to have high electrical conductivity and are generally made from a base material of copper or copper alloys. Copper and copper alloys are, however, easily corroded by oxygen or corrosive gases in the air. For anti-rust and anti-corrosion purposes, formation of coating layers of multi-layered nickel plating and gold plating films on the base material has been examined.

Patent Document 1 shows, for example, that an electroless nickel film as an underlayer is formed on the base material of a connection terminal and an electroless displacement gold plating film and an electroless reductional gold plating film are formed in this order on the underlayer.

Patent Document 1: Japanese Patent Application Laid-Open No. 2010-37603

## SUMMARY

The coating layers in Patent Document 1 are made using electrons produced in the corrosion reaction of a nickel plating film, the electrons reducing gold ions in the plating solution through electroless displacement gold plating. The nickel plating film is therefore easily corroded, which can lead to defects in the gold plating films. The gold plating films can be made thick enough for preventing such defects in them, but this will readily increase the manufacturing cost of the coating layers because gold is generally expensive.

With a thinner or no gold plating film formed, the nickel plating film is exposed as the outermost layer, which will lower corrosion resistance. The lowered corrosion resistance will reduce the functionality of the conductor as a signal transfer unit and increase contact resistance in electrical connection with external apparatuses. In other words, reliability in electrical connection with external apparatuses for sending and receiving electrical signals to and from these apparatuses is compromised.

In view of the foregoing, some aspects of the present invention are directed to provide a coating having sufficient corrosion resistance and connection reliability and also to an electronic component including a signal transfer unit provided with this coating thereby having sufficient corrosion resistance and connection reliability.

An aspect of the present invention provides a coating provided to a conductor, the coating including a palladium layer having a crystal plane whose orientation rate is 65% or more.

An aspect of the present invention provides a coating provided to a conductor, the coating including a palladium layer having a crystal plane whose orientation rate is 65% or more.

In the coating, the palladium layer has a crystal plane whose orientation rate is 65% or more, which means 65% or more of the crystal planes of the palladium layer is aligned to this crystal plane. The conductor provided with the coating,

therefore, has superior corrosion resistance and thus has superior reliability in electrical connection with external apparatuses.

Preferably the crystal plane whose orientation rate is 65% or more in the coating is the (111) plane or (200) plane. This can allow the coating to have a reduced stress remaining in the palladium layer, while providing corrosion resistance and reliability in electrical connection with external apparatuses.

Preferably the palladium layer in the coating contains phosphorus in a concentration ranging from 0.5% by mass to 2.5% by mass. This can allow the coating to have enhanced abrasion resistance by making the crystal of the palladium layer finer and denser, while providing more superior corrosion resistance and reliability in electrical connection with external apparatuses.

Preferably the coating further includes a gold layer on the opposite surface of the palladium layer to the conductor. This can allow the coating to provide corrosion resistance and reliability in electrical connection with external apparatuses in even higher levels.

Preferably the coating also includes a metal underlayer between the palladium layer and the conductor. With a stabilized state of the underlayer of the palladium layer, the palladium layer can be made thinner, while providing superior corrosion resistance and reliability in electrical connection with external apparatuses.

In particular, the metal underlayer preferably includes at least one metal selected from the group consisting of Ni, Sn, Fe, Co, Zn, Rh, Ag, Pt, Au, Pb, and Bi. With a nickel underlayer serving as the metal underlayer for stabilizing the state of the underlayer of the palladium layer without fail, the palladium layer can be made thinner, while maintaining superior corrosion resistance and reliability in electrical connection with external apparatuses.

Another aspect of the present invention provides an electronic component including a signal transfer unit having the coating described above and a conductor coated with the coating. This signal transfer unit has the conductor coated with the coating having the features described above, which can provide an electronic component including a signal transfer unit having sufficient corrosion resistance and connection reliability.

Some aspects of the present invention can provide a coating having sufficient corrosion resistance and connection reliability and also provide an electronic component including a signal transfer unit provided with this coating thereby having sufficient corrosion resistance and connection reliability.

## BRIEF DESCRIPTION OF DRAWINGS

FIG. 1 is a perspective view schematically showing a preferred embodiment of an electronic component including a signal transfer unit having a coating;

FIG. 2 is a sectional view schematically showing the signal transfer unit in FIG. 1 along line II-II;

FIG. 3 is a sectional view schematically showing another embodiment of a signal transfer unit having a coating;

FIG. 4 is a sectional view schematically showing yet another embodiment of a signal transfer unit having a coating;

FIG. 5 is a sectional view schematically showing still another embodiment of a signal transfer unit having a coating; and

FIG. 6 is an X-ray diffraction chart of a signal transfer unit in Example 6.

## DESCRIPTION OF EMBODIMENTS

Preferred embodiments are described hereinafter with reference to the accompanying drawings. The same or equiva-

lent components are given the same reference numerals in the drawings, and the description relating thereto will be omitted.

As shown in FIG. 1, an electronic component **100** according to one embodiment includes a signal transfer unit **10** on a base **70**. Examples of the electronic component **100** include active components such as transistors, integrated circuits, and antennas; passive components such as capacitors, inductors, and filters; and circuit components such as printed wiring boards and module board.

The signal transfer unit **10** provided to the electronic component **100** serves as a connection terminal connected to other members through contact, bonding wiring, or soldering or as an open terminal, thereby providing a pathway for electrical signals or power supply for operating the electronic component **100**. The signal transfer unit **10** may serve as a connection terminal for supplying the electronic component **100** with power supply potential or grounding potential or as a signal terminal for inputting or outputting signals. In this manner, the signal transfer unit **10** can be used for various applications that require corrosion resistance and connection reliability.

As shown in FIG. 2, the signal transfer unit **10** according to the present embodiment includes a conductor **50** and a coating **1** that coats (is provided on) the conductor **50**. The coating **1** according to the present embodiment is a coating layer for preventing corrosion of the conductor **50**. The coating **1** has a layered structure of a palladium layer **12**.

The palladium layer **12** in the coating **1** according to the present embodiment has a crystal plane whose orientation rate is 65% or more. In the palladium layer **12** having a crystal plane whose orientation rate is 65% or more, many crystal planes are aligned to this crystal plane. This leads to fewer crystal grain boundaries having crystal planes, the boundaries can often become the trigger of corrosion. As a result, a coating having superior corrosion resistance can be provided. In addition, the state of the surface of the coating is stabilized at the atomic level because many crystal planes are aligned to the crystal plane whose orientation rate is 65% or more. The stabilized contact surface has a reduced contact resistance. As a result, a coating having superior corrosion resistance and high connection reliability can be provided.

Crystal planes of the palladium layer **12** and their orientation rates can be analyzed through the X-ray diffraction analysis or electron diffraction analysis, for example, of the palladium layer **12**. More specifically, the orientation rates of palladium crystal planes, namely, the (111) plane, the (200) plane, the (220) plane, the (311) plane, the (222) plane, the (400) plane, the (331) plane, and the (420) plane, are determined as follows when their diffraction peaks are observed, whereas the orientation rates of these crystal planes are set 0% when their diffraction peaks are substantially not observed.

The orientation rates of the crystal planes can be expressed in percentage by the ratio of the diffraction peak intensity of each of the crystal planes to the sum of the diffraction peak intensities of all the crystal planes whose diffraction peaks are observed. The palladium layer **12** according to the present embodiment has a crystal plane whose orientation rate is 65% or more. As this crystal plane has an orientation rate of 65% or more, the sum of the orientation rates of the other crystal planes is 35% at most. Thus, the crystal plane whose orientation rate is 65% or more in the palladium layer **12** can be identified uniquely.

In the X-ray diffraction spectrum shown in FIG. 6, assuming that the diffraction peaks of the (111) plane and the (200) plane, which are palladium crystal planes, are observed, the diffraction peak intensity of the (111) plane is denoted as  $I(111)$  and the diffraction peak intensity of the (200) plane is

denoted as  $I(200)$ . In this case, the relation  $I(111) > I(200)$  holds true. The orientation rate  $R$  of each crystal plane is defined by:  $R = I(111) / \{I(111) + I(200)\}$ . The crystal plane with the largest orientation rate is the (111) plane.

The orientation rate of the crystal plane whose orientation rate is 65% or more in the palladium layer **12** is preferably 70% or more. In the palladium layer having a crystal plane whose orientation rate is 70% or more, even more crystal planes are aligned to this crystal plane, whereby the advantageous effects described above can be provided sufficiently.

The crystal plane whose orientation rate is 65% or more in the palladium layer **12** is preferably any one of the (111) plane and the (200) plane. Any one of the (111) plane and the (200) plane serving as the crystal plane whose orientation rate is 65% or more can allow the coating to have a reduced stress remaining in the palladium layer **12**, while providing superior corrosion resistance and high connection reliability.

The palladium layer **12** preferably contains phosphorus in a concentration ranging from 0.5% by mass to 2.5% by mass. Inclusion of phosphorus in the palladium layer **12** in a concentration of 0.5% by mass or more makes the crystal finer and denser, whereby the corrosion resistance and abrasion resistance of the palladium layer **12** are enhanced. Inclusion of phosphorus in the palladium layer **12** in a concentration above 2.5% by mass, however, makes the surface of the coating less stable at the atomic level, which makes it difficult to fully achieve the advantageous effects of the embodiment.

The thickness of the palladium layer **12** preferably ranges from 0.05  $\mu\text{m}$  to 0.5  $\mu\text{m}$ . The thickness below 0.05  $\mu\text{m}$  provides an insufficient coating of the palladium layer **12** for the conductor **50**, which can fail to provide sufficient corrosion resistance. The thickness exceeding 0.5  $\mu\text{m}$ , which can increase the manufacturing cost, tends to make a limited contribution to the corrosion resistance.

Examples of the conductor **50** include at least one selected from copper (Cu), silver (Ag), and their alloys. The conductor **50** preferably contains copper from the viewpoint of reducing the manufacturing cost of the signal transfer unit **10**. Examples of the conductor **50** include a conductive terminal functioning as the signal transfer unit **10**. A copper terminal provided to a wiring board in the electronic component **100** or an antenna signal transfer unit can be given as an example.

A method for making the coating **1** according to the present embodiment will now be described. The method for making the coating **1** includes a conductor pre-processing step of performing pre-processing on the surface of the conductor **50** and a palladium plating step of performing palladium plating to provide a palladium plating film serving as the palladium layer **12**.

In the conductor pre-processing step, the conductor **50** is etched and then activated. The conductor pre-processing can include, but is not limited to immersion in an etchant or an activator liquid. The pre-processing on the surface of the conductor **50** can affect the coating or crystalline property of the palladium layer **12** provided later on the conductor **50**. An appropriate adjustment in liquid composition, temperature, processing time, and other conditions in the etching and activation can therefore allow the palladium layer **12** provided later to have a crystal plane whose orientation rate is 65% or more.

In the palladium plating step, palladium plating is performed to provide the palladium layer **12** of a palladium plating film on the conductor **50**, which has been pre-processed. The palladium plating can include, but is not limited to, electroless palladium plating such as reductional palladium plating and displacement palladium plating. One of these plating processing methods can be selected as appro-

priate to make a desired palladium layer 12. From the viewpoint of making a crystal plane whose orientation rate is 65% or more, reductional palladium plating is preferably selected.

Examples of palladium compounds contained in the plating solution for reductional palladium plating include aqueous solutions containing palladium sulfate, palladium nitrate, palladium acetate, palladium chloride, palladium bromide, palladium hydroxide, palladium cyanide, diamminedichloropalladium, diamminedinitropalladium, tetraamminepalladium dichloride, tetraamminepalladium dibromide, tetrachloropalladate, tetracyanopalladate, tetrathiocyanatopalladate, and tetrabromopalladate. Examples of salts include sodium salts, potassium salts, and ammonium salts. An appropriate adjustment of the concentration of phosphorus in the plating solution for making a reductional palladium plating film can allow the reductional palladium plating film to have a crystal plane whose orientation rate is 65% or more. The reductional palladium plating film is made through the phenomenon in which palladium ions gain electrons in the plating solution, the electrons being emitted in the oxidation reaction of a material with a reduction action, i.e., reducing agent, in the plating solution. In other words, the plating solution contains the reducing agent.

Examples of the reducing agent contained in the plating solution include phosphorous compounds such as hypophosphorous acid, phosphorous acid, and salts thereof (e.g., sodium salts, potassium salts, and ammonium salts); carbon compounds such as formalin, formic acid, and salts thereof; boron compounds such as borofluorides and dimethylamine borane; and sulfur compounds such as thiosulfuric acid, peroxide sulfuric acid, and salts thereof. Instead, the reducing agent may be polyvalent metal ions such as divalent tin ions, divalent cobalt ions, and divalent iron ions, for example.

The reductional palladium plating film made through the reduction reaction is deposited on the conductor 50, which has been pre-processed, by electrons emitted from the reducing agent. If the reducing agent contains phosphorus in this process, the phosphorus is codeposited in the reductional palladium plating film. These actions can allow the reductional palladium plating film to have a crystal plane whose orientation rate is 65% or more. In addition, the reductional palladium plating film can be allowed to have a crystal plane whose orientation rate is 65% or more and the concentration of phosphorus in the plating solution can be adjusted by changing the types of palladium compounds contained in the plating solution and of the reducing agent containing phosphorus and changing their contents in the plating solution.

In this manner, phosphorus contained in the compounds serving as the reducing agent is codeposited in the palladium plating film made through the reduction reaction, whereby the corrosion resistance of the palladium plating film can be enhanced. The method for making the palladium layer 12 is not limited to the method described above and may be sputtering or vapor deposition, for example.

A coating according to another embodiment of the present invention will now be described.

FIG. 3 is a sectional view schematically showing a signal transfer unit having a coating according to the present invention. This signal transfer unit 20 shown in FIG. 3 is a signal transfer unit in an electronic component and includes the conductor 50 and a coating 2 that coats (is provided on) the conductor 50. The coating 2 according to the present embodiment is a coating layer for preventing corrosion of the conductor 50. The coating 2 has a multi-layered structure of the palladium layer 12 and a gold layer 14 deposited in this order from the conductor 50. In other words, the coating 2 according to the present embodiment differs from the coating 1

according to the above-described embodiment in that the coating 2 includes the gold layer 14 on the opposite surface of the palladium layer 12 to the conductor 50. The components of the coating 2 other than the gold layer 14 can be the same as those of the coating 1.

The gold layer 14 is preferably a gold plating film made through gold plating. Providing this gold layer 14 can allow the coating to have even higher reliability in electrical connection with external apparatuses by further reducing the contact resistance on the surface of the coating 2, while maintaining sufficient corrosion resistance.

The thickness of the gold layer 14 is preferably 0.1  $\mu\text{m}$  or less, and more preferably ranges from 0.01  $\mu\text{m}$  to 0.08  $\mu\text{m}$  from the viewpoint of further reducing the contact resistance.

15 The thickness below 0.01  $\mu\text{m}$  tends to fail to achieve the effect of further reducing the contact resistance. The thickness exceeding 0.1  $\mu\text{m}$ , which can increase the manufacturing cost, tends to make a limited contribution to the contact resistance.

20 The palladium layer 12 according to the present embodiment has a crystal plane whose orientation rate is 65% or more and many crystal planes are aligned to this crystal plane as described above. This leads to fewer crystal grain boundaries having crystal planes, the boundaries can often become the trigger of corrosion. The state of the surface of the palladium layer 12 to which the gold layer 14 is provided is thus stabilized at the atomic level. As a result, the gold layer 14 is evenly and firmly provided even with a small thickness. This can allow the coating to have even higher reliability in electrical connection with external apparatuses, while maintaining sufficient corrosion resistance.

25 A method for making the coating 2 according to the present embodiment will be described. The method for making the coating 2 includes a conductor pre-processing step of performing pre-processing on the surface of the conductor 50, a palladium plating step of performing palladium plating to provide the palladium layer 12, and a gold plating step of performing gold plating on the palladium layer 12 to provide a gold plating film serving as the gold layer 14 on the palladium layer 12. This method can be performed in the same manner as the method for making the coating 1 described above except for the gold plating step, and thus the gold plating step will now be described.

30 In the gold plating step, electroless gold plating such as displacement gold plating and reductional gold plating is performed to provide the gold layer 14 of a gold plating film on the surface of the palladium layer 12. The gold plating film can be provided through a known method using a commercially available electroless gold plating solution. The method for making the gold layer 14 is not limited to the method described above and may be sputtering or vapor deposition, for example.

35 A coating according to yet another embodiment of the present invention will now be described.

40 FIG. 4 is a sectional view schematically showing a signal transfer unit having a coating according to the present invention. This signal transfer unit 30 shown in FIG. 4 is a signal transfer unit in an electronic component and includes the conductor 50 and a coating 3 that coats (is provided on) the conductor 50. The coating 3 according to the present embodiment is a coating layer for preventing corrosion of the conductor 50. The coating 3 has a multi-layered structure of a metal underlayer 16 and the palladium layer 12 deposited in this order from the conductor 50. In other words, the coating 3 according to the present embodiment differs from the coating 1 according to the above-described embodiment in that the coating 3 includes the metal underlayer 16 between the

conductor 50 and the palladium layer 12. The components of the coating 3 other than the metal underlayer 16 can be the same as those of the coating 1.

The metal underlayer 16 is preferably a metal plating film, made through electroless metal plating. The used metal is at least one metal selected from the group consisting of nickel (Ni), tin (Si), iron (Fe), cobalt (Co), zinc (Zn), rhodium (Rh), silver (Ag), platinum (Pt), gold (Au), lead (Pb), and bismuth (Bi) and still has the function of isolation. The metal underlayer can be made from an alloy containing at least one of these metal elements.

The metal underlayer 16 is more preferably a nickel plating film made through electroless nickel plating. Providing this metal underlayer 16 stabilizes the state of the base underlying the palladium layer 12. This can make the palladium layer 12 thin, while maintaining sufficient corrosion resistance. As a result, the amount of palladium used is reduced, which can further reduce the manufacturing cost of the coating 3. The thickness of the metal underlayer 16 is preferably 1  $\mu\text{m}$  or more from the viewpoint of sufficiently reducing the manufacturing cost. When the signal transfer unit 30 has the function of using high-frequency radio waves for transferring signals, the signals tend to be transferred in the outermost layer of the conductor 50. In this case, arranging the metal underlayer 16 with a low electrical conductivity adjacent to the conductor 50 can easily increase loss. In this sense, the thickness of the metal underlayer 16 is preferably 10  $\mu\text{m}$  or less. The thickness of the metal underlayer 16 is preferably adjusted as appropriate depending on the thickness of the conductor 50 and the frequencies of signals. Using Sn or the other metal elements (Fe, Co, Zn, Ag, Pt, Au, Pb, and Bi) besides Ni can provide similar advantageous effects.

A method for making the coating 3 according to the present embodiment will be described. In the present embodiment, the metal underlayer 16 is of nickel. The method for making the coating 3 includes a conductor pre-processing step of performing pre-processing on the surface of the conductor 50, a nickel plating step of performing electroless nickel plating to provide a nickel plating film serving as the metal underlayer 16, and a palladium plating step of performing palladium plating on the metal underlayer 16 to provide the palladium layer 12. This method can be performed in the same manner as the method for making the coating 1 described above except for the nickel plating step, and thus the nickel plating step will now be described.

In the nickel plating step, electroless nickel plating is performed to provide the metal underlayer 16 of an electroless nickel plating film on the conductor 50. Subsequently, palladium plating is performed to provide the palladium layer 12 to make the coating 3 as in the method for making the coating 1. The method for making the metal underlayer 16 is not limited to the method described above and may be sputtering or vapor deposition, for example.

Some preferred embodiments of the present invention are described above, but the present invention is not limited to these embodiments in any manner. For example, whereas the above-described embodiments provide the gold layer 14 on the opposite surface of the palladium layer 12 to the conductor 50 or provide the metal underlayer 16 between the conductor 50 and the palladium layer 12, the gold (Au) layer 14 may be provided on the opposite surface of the palladium layer 12 to the conductor 50 and the metal underlayer 16 may be provided between the conductor 50 and the palladium layer 12 as shown in FIG. 5.

FIG. 5 is a sectional view schematically showing a signal transfer unit having a coating according to the present embodiment.

The signal transfer unit 30 shown in FIG. 5 includes the conductor 50 and a coating 4 that coats the conductor 50. The coating 4 according to the present embodiment is a coating layer for preventing corrosion of the conductor 50. The coating 4 has a multi-layered structure of the metal underlayer 16, the palladium layer 12, and the gold layer 14 deposited in this order from the conductor 50. In other words, the coating 4 according to the present embodiment differs from the coating 3 according to the above-described embodiment shown in FIG. 4 in that the coating 4 includes the gold layer 14 on the palladium layer 12. The components of and the method for making the coating 4 can be the same as those of the coating 1, the coating 2, and the coating 3.

This structure can allow the coating to have sufficient corrosion resistance and high connection reliability by further reducing the contact resistance, while reducing the manufacturing cost of the coating with a reduced thickness of the palladium layer 12. The coating including the gold layer 14 on the opposite surface of the palladium layer 12 to the conductor 50 and the metal underlayer 16 between the conductor 50 and the palladium layer 12 can be provided by, for example, performing the above-described electroless nickel plating, palladium plating, and gold plating on the conductor 50 in this order.

For example, the conductor 50 may be partially in contact with a sealing resin material or a resist material provided to the electronic component 100. In this case, the part of the conductor 50 in contact with the sealing resin material or the resist material is not necessarily provided with the coating according to the present invention. The coating according to the present invention needs to be provided at least to another part of the conductor 50 not in contact with the sealing resin material or the resist material, e.g., the coating is provided partially on the opposite surface of the conductor 50 to the base 70 or a side of the conductor 50.

## EXAMPLES

The invention will be described in greater detail, using some examples and comparative examples. It is understood that the present invention is not limited to the examples below.

### Preparation of Signal Transfer Units Having Coating

#### Example 1

##### Etching Step

A piece of commercially available copper foil (thickness: 20  $\mu\text{m}$ ) was bonded to a commercially available glass epoxy substrate (height  $\times$  width  $\times$  thickness: 30 mm  $\times$  30 mm  $\times$  0.5 mm) with adhesive to produce a copper-foil-covered substrate (conductor). An etchant (temperature: 30°C.) of the composition in Table 1 was prepared separately. The conductor was immersed in the etchant for one minute to etch the surface of the conductor. After the etching, the conductor was washed with water to provide an etched conductor. The etchant contained sodium persulfate and sulfuric acid (98% by mass).

TABLE 1

| Composition                 | Content |
|-----------------------------|---------|
| Sodium persulfate           | 100 g/L |
| Sulfuric acid (98% by mass) | 30 mL/L |

## Activation Step

An activator liquid (temperature: 30° C.) of the composition in Table 2 was prepared. The conductor etched as described above was immersed in an aqueous solution (temperature: 30° C.) prepared by diluting 30-ml sulfuric acid (98%) with water for 30 seconds and the conductor was then immersed in the activator liquid of Table 2 for one minute to activate the surface of the conductor. After the activation, the conductor was washed with water to provide an activated conductor. The activator liquid contained palladium sulfate and ammonium nitrate.

TABLE 2

| Composition       | Content                                 |
|-------------------|-----------------------------------------|
| Palladium sulfate | 1 g/L (on a palladium conversion basis) |
| Ammonium nitrate  | 30 g/L                                  |

## Palladium Plating Step

An electroless palladium plating solution (temperature: 55° C.; pH: 6.0) of the composition in Table 3 was prepared. The conductor activated as described above was immersed in the electroless palladium plating solution of Table 3 for 10 minutes to provide a palladium plating film. After the palladium plating, the conductor with the palladium plating film thereon was washed with water to provide a coating having a layered structure of a palladium layer on the conductor. This sample was a signal transfer unit in Example 1. The electroless palladium plating solution contained diammine palladium nitrite, disodium ethylenediaminetetraacetate, sodium hydrogen phosphite, and sodium formate.

TABLE 3

| Composition                          | Content                                   |
|--------------------------------------|-------------------------------------------|
| Diammine palladium nitrite           | 1.5 g/L (on a palladium conversion basis) |
| Disodium ethylenediaminetetraacetate | 10 g/L                                    |
| Sodium hydrogen phosphite            | 3 g/L                                     |
| Sodium formate                       | 10 g/L                                    |

## Example 2

A conductor provided with a palladium layer was made in the same manner as in Example 1.

## Gold Plating Step

An electroless gold plating solution (temperature: 80° C.; pH: 5.0) of the composition in Table 4 was prepared. The conductor with a nickel underlayer and a palladium layer deposited in this order as described above was immersed in the gold plating solution of Table 4 for 10 minutes to provide a gold plating film. After the gold plating, the conductor with the gold plating film thereon was washed with water to provide a coating having a multi-layered structure of the palladium layer and the gold layer deposited in this order on the conductor. This sample was a signal transfer unit in Example 2. The electroless gold plating solution contained potassium gold cyanide, sodium cyanide, and sodium carbonate.

TABLE 4

| Composition            | Content                            |
|------------------------|------------------------------------|
| Potassium gold cyanide | 2 g/L (on a gold conversion basis) |
| Sodium cyanide         | 30 g/L                             |
| Sodium carbonate       | 20 g/L                             |

## Example 3

A coating having a layered structure of a palladium layer was provided on a conductor in the same manner as in Example 1, except that the palladium plating solution of Table 3 was replaced with a palladium plating solution (temperature: 55° C.; pH: 6.0) of the composition in Table 5 in the palladium plating step. This sample was a signal transfer unit in Example 3. The palladium plating solution contained diammine palladium nitrite, disodium ethylenediaminetetraacetate, and sodium hydrogen phosphite.

TABLE 5

| Composition                          | Content                                   |
|--------------------------------------|-------------------------------------------|
| Diammine palladium nitrite           | 1.0 g/L (on a palladium conversion basis) |
| Disodium ethylenediaminetetraacetate | 10 g/L                                    |
| Sodium hydrogen phosphite            | 20 g/L                                    |

## Example 4

A coating having a multi-layered structure of a palladium layer and a gold layer deposited in this order was provided on a conductor in the same manner as in Example 2, except that the palladium plating solution of Table 3 was replaced with a palladium plating solution (temperature: 55° C.; pH: 6.0) of the composition in Table 5 in the palladium plating step. This sample was a signal transfer unit in Example 4.

## Example 5

A coating having a layered structure of a palladium layer was provided on a conductor in the same manner as in Example 1, except that the palladium plating solution of Table 3 was replaced with a palladium plating solution (temperature: 60° C.; pH: 7.0) of the composition in Table 6 and the processing time for immersing the conductor in the palladium plating solution was changed from 10 minutes to 5 minutes in the palladium plating step. This sample was a signal transfer unit in Example 5. The palladium plating solution contained tetraammine palladium dichloride, disodium ethylenediaminetetraacetate, and sodium phosphite.

TABLE 6

| Composition                          | Content                                   |
|--------------------------------------|-------------------------------------------|
| Tetraammine palladium dichloride     | 0.7 g/L (on a palladium conversion basis) |
| Disodium ethylenediaminetetraacetate | 20 g/L                                    |
| Sodium phosphite                     | 100 g/L                                   |

## Example 6

A coating having a layered structure of a palladium layer was provided on a conductor in the same manner as in Example 5, except that the processing time for immersing the conductor in the palladium plating solution in Table 6 was changed from 5 minutes to 20 minutes in the palladium plating step. This sample was a signal transfer unit in Example 6.

## Example 7

A coating having a layered structure of a palladium layer was provided on a conductor in the same manner as in

## 11

Example 5, except that the processing time for immersing the conductor in the palladium plating solution in Table 6 was changed from 5 minutes to 40 minutes in the palladium plating step. This sample was a signal transfer unit in Example 7.

## Example 8

A coating having a multi-layered structure of a palladium layer and a gold layer deposited in this order was provided on a conductor in the same manner as in Example 2, except that the palladium plating solution of Table 3 was replaced with a palladium plating solution (temperature: 60° C.; pH: 7.0) of the composition in Table 6 and the processing time for immersing the conductor in the palladium plating solution was changed from 10 minutes to 20 minutes in the palladium plating step. This sample was a signal transfer unit in Example 8.

## Example 9

## Etching Step and Activation Step

An etched conductor was made in the same manner as in the above-described example 1. The conductor was immersed in a commercially available activator liquid (from Uyemura & Co., Ltd.; trade name: AT-450; temperature: 30° C.) for one minute to perform activation. After the activation, the conductor was washed with water to provide an activated conductor.

## Nickel Plating Step

An electroless nickel plating solution (temperature: 85° C.; pH: 4.5) of the composition in Table 7 was prepared. The conductor activated as described above was immersed in the electroless nickel plating solution of Table 7 for 30 minutes to provide a nickel plating film. After the nickel plating, the conductor was washed with water to provide the conductor with a nickel underlayer thereon. The electroless nickel plating solution contained nickel sulfate, sodium hypophosphite, sodium citrate, and ammonium chloride.

TABLE 7

| Composition          | Content |
|----------------------|---------|
| Nickel sulfate       | 20 g/L  |
| Sodium hypophosphite | 15 g/L  |
| Sodium citrate       | 30 g/L  |
| Ammonium chloride    | 30 g/L  |

## Palladium Plating Step

The palladium plating solution (temperature: 60° C.; pH: 7.0) of the composition in Table 6 was prepared. The conductor provided with the nickel underlayer as described above was immersed in the electroless palladium plating solution of Table 6 for 5 minutes to provide a palladium plating film. After the palladium plating, the conductor was washed with water to provide the conductor with the nickel underlayer and the palladium layer thereon.

## Gold Plating Step

An electroless gold plating solution (temperature: 80° C.; pH: 5.0) of the composition in Table 4 was prepared. The conductor with the nickel underlayer and the palladium layer deposited in this order as described above was immersed in the gold plating solution of Table 4 for 10 minutes to provide a gold plating film. After the gold plating, the conductor was washed with water to provide a coating having a multi-layered structure of the nickel underlayer, the palladium layer,

## 12

and the gold layer in this order on the conductor. This sample was a signal transfer unit in Example 9.

## Example 10

A coating having a layered structure of a palladium layer was provided on a conductor in the same manner as in Example 1, except that the palladium plating solution of Table 3 was replaced with a palladium plating solution (temperature: 65° C.; pH: 7.0) of the composition in Table 8 and the processing time for immersing the conductor in the palladium plating solution was changed from 10 minutes to 20 minutes in the palladium plating step. This sample was a signal transfer unit in Example 10. The palladium plating solution contained ammonium tetrachloropalladate, ethylenediamine, and sodium hypophosphite.

TABLE 8

| Composition                   | Content                                 |
|-------------------------------|-----------------------------------------|
| Ammonium tetrachloropalladate | 1 g/L (on a palladium conversion basis) |
| Ethylenediamine               | 15 g/L                                  |
| Sodium hypophosphite          | 1 g/L                                   |

## Example 11

A coating having a multi-layered structure of a palladium layer and a gold layer deposited in this order was provided on a conductor in the same manner as in Example 2, except that the palladium plating solution of Table 3 was replaced with a palladium plating solution (temperature: 65° C.; pH: 7M) of the composition in Table 8 and the processing time for immersing the conductor in the palladium plating solution was changed from 10 minutes to 20 minutes in the palladium plating step. This sample was a signal transfer unit in Example 11.

## Example 12

A coating having a multi-layered structure of a palladium layer and a gold layer deposited in this order was provided on a conductor in the same manner as in Example 2, except that the palladium plating solution of Table 3 was replaced with a palladium plating solution (temperature: 65° C.; pH: 7.0) of the composition in Table 9 and the processing time for immersing the conductor in the palladium plating solution was changed from 10 minutes to 20 minutes in the palladium plating step. This sample was a signal transfer unit in Example 12. The palladium plating solution contained ammonium tetrachloropalladate, ethylenediamine, and sodium hypophosphite.

TABLE 9

| Composition                   | Content                                   |
|-------------------------------|-------------------------------------------|
| Ammonium tetrachloropalladate | 0.7 g/L (on a palladium conversion basis) |
| Ethylenediamine               | 20 g/L                                    |
| Sodium hypophosphite          | 2 g/L                                     |

## Example 13

## Etching Step

An etched conductor was provided in the same manner as in the above-described example 1.

13

**Tin Plating Step**

An electroless tin plating solution (temperature: 30° C.; pH: 1.5) of the composition in Table 13 below was prepared. The conductor etched as described above was immersed in the electroless tin plating solution of Table 13 for 30 minutes to provide a tin plating film. After the tin plating, the conductor was washed with water to provide the conductor with a tin underlayer thereon. The electroless tin plating solution contained tin methanesulfonate, methanesulfonic acid, thiourea, and an additive.

**Palladium Plating Step**

A palladium plating solution (temperature: 65° C.; pH: 7.0) of the composition in Table 8 was prepared. A conductor provided with a tin underlayer as described above was immersed in the electroless palladium plating solution of Table 8 for 20 minutes to provide a palladium plating film. After the palladium plating, the conductor was washed with water to provide a coating having a multi-layered structure of the tin underlayer and the palladium layer in this order on the conductor. This sample was a signal transfer unit in Example 13.

**Example 14**

A conductor with a tin underlayer and a palladium layer deposited in this order was prepared in the same manner as in Example 13.

**Gold Plating Step**

An electroless gold plating solution (temperature: 80° C.; pH: 5.0) of the composition in Table 4 was prepared. A conductor with a tin underlayer and a palladium layer deposited in this order as described above was immersed in the gold plating solution of Table 4 for 10 minutes to provide a gold plating film. After the gold plating, the conductor with the gold plating film thereon was washed with water to provide a coating having a multi-layered structure of the tin underlayer, the palladium layer, and the gold layer in this order on the conductor. This sample was a signal transfer unit in Example 14.

**Example 15**

A coating having a multi-layered structure of a tin underlayer, a palladium layer, and a gold layer in this order was provided on a conductor in the same manner as in Example 14, except that the palladium plating solution of Table 8 was replaced with the palladium plating solution (temperature: 65° C.; pH: 7.0) of the composition in Table 9 in the palladium plating step. This sample was a signal transfer unit in Example 15.

**Comparative Example 1**

A coating having a multi-layered structure of a nickel underlayer and a palladium layer deposited in this order was provided on a conductor in the same manner as in Example 9, except that the palladium plating solution of Table 6 was replaced with a palladium plating solution (temperature: 50° C.; pH: 7.5) of the composition in Table 10 and the processing time for immersing the conductor in the palladium plating solution was changed from 5 minutes to 10 minutes in the palladium plating step, and no gold plating was performed. This sample was a signal transfer unit in Comparative Example 1. The palladium plating solution contained palladium sulfate, ethylenediamine, sodium formate, and sodium hypophosphate.

14

TABLE 10

| Composition          | Content                                 |
|----------------------|-----------------------------------------|
| Palladium sulfate    | 1 g/L (on a palladium conversion basis) |
| Ethylenediamine      | 20 g/L                                  |
| Sodium formate       | 15 g/L                                  |
| Sodium hypophosphate | 1 g/L                                   |

**Comparative Example 2**

A coating having a multi-layered structure of a nickel underlayer and a palladium layer in this order was provided on a conductor in the same manner as in Comparative Example 1, except that the palladium plating solution of Table 10 was replaced with a palladium plating solution (temperature: 50° C.; pH: 7.5) of the composition in Table 11 in the palladium plating step. This sample was a signal transfer unit in Comparative Example 2. The palladium plating solution contained palladium sulfate, ethylenediamine, sodium formate, and sodium hypophosphate.

TABLE 11

| Composition          | Content                                 |
|----------------------|-----------------------------------------|
| Palladium sulfate    | 1 g/L (on a palladium conversion basis) |
| Ethylenediamine      | 20 g/L                                  |
| Sodium formate       | 15 g/L                                  |
| Sodium hypophosphate | 2 g/L                                   |

**Comparative Example 3**

A coating having a multi-layered structure of a nickel underlayer and a palladium layer in this order was provided on a conductor in the same manner as in Comparative Example 1, except that the palladium plating solution of Table 10 was replaced with a palladium plating solution (temperature: 70° C.; pH: 5.5) of the composition in Table 12 in the palladium plating step. This sample was a signal transfer unit in Comparative Example 3. The palladium plating solution contained palladium chloride, ethylenediamine, and sodium hypophosphate.

TABLE 12

| Composition          | Content                                 |
|----------------------|-----------------------------------------|
| Palladium chloride   | 1 g/L (on a palladium conversion basis) |
| Ethylenediamine      | 10 g/L                                  |
| Sodium hypophosphate | 5 g/L                                   |

The electroless tin plating solution used for tin (Sn) plating in Examples 13 to 15 had the following composition.

TABLE 13

| Composition          | Content |
|----------------------|---------|
| Tin methanesulfonate | 30 g/L  |
| Methanesulfonic acid | 100 g/L |
| Thiourea             | 70 g/L  |

**Evaluation of Signal Transfer Units Having Coating**

The crystalline property of the palladium layer in the coating for the signal transfer unit in each of the examples and comparative examples was evaluated using an X-ray diffractometer. Specifically, the orientation rate of each of the crystal

planes whose diffraction peaks attributable to palladium crystal planes were observed was determined. Of the crystal planes whose diffraction peaks were observed, the crystal plane with the largest orientation rate and its orientation rate were identified. For example, FIG. 6 is an X-ray diffraction chart of the signal transfer unit in Example 6 using a CuK $\alpha$  X-ray source.

As a result of the X-ray diffraction, a diffraction peak attributable to a crystal plane of the conductor (copper foil) was observed, and diffraction peaks attributable to the (111) plane and the (200) plane, which are palladium crystal planes, were observed. Substantially no diffraction peaks attributable to the other palladium crystal planes were observed. The orientation rates of the crystal planes were determined in percentage by the ratio of the diffraction peak intensity of each of the crystal planes to the sum of the diffraction peak intensities of the (111) plane and the (200) plane, whose diffraction peaks were observed. As a result, the crystal plane with the largest orientation rate was the (111) plane and its orientation rate was 85%. Table 14 lists the results in the examples and comparative examples. Samples whose diffraction peaks attributable to any palladium crystal planes were substantially not observed are marked with "Amorphous".

Each of the signal transfer units in the examples and comparative examples was cut along the layered direction of the coating. The cut surface was observed under a transmission electron microscope (TEM) to determine the thickness of each layer in the layer structure of the coating. The cut surface was also analyzed with an energy dispersive X-ray spectrometer (EDS) to determine the concentration of phosphorus in each palladium layer. The results are listed in Table 14.

Contact resistance was determined in the following manner to evaluate the connection reliability of each of the signal transfer units in the examples and comparative examples. Commercially available contact probes were prepared that were finished with gold plating on a nickel base. Each of the probes had a spherical tip ( $R=0.6$  mm) serving as a contact tip. The resistance of the contact probe was determined to be 11.0 m $\Omega$  through the four-terminal method with the contact tip connected to one Kelvin probe and the other end of the contact probe to the contact tip connected to the other Kelvin probe.

Then, with one Kelvin probe connected to the signal transfer unit and the other Kelvin probe connected to the opposite end of the contact probe to the contact tip, the contact tip of the contact probe was brought into contact with the surface of the signal transfer unit with a 1-N pressing force using a jig. Under this state, 10-mA current was applied to make a series resistance circuit with which the resistance of the contact probe and the sum of the contact resistance and the resistance of the signal transfer unit were determined through the four-terminal method. Separately, the resistance of the signal

transfer unit was determined through the four-terminal method, whereby sufficiently low resistances (less than 0.1 m $\Omega$ ) were obtained in all the examples and comparative examples. The contact resistance was finally determined by subtracting the resistance of the contact probe (11.0 m $\Omega$ ) from the sum.

The connection reliability was evaluated as follows: samples whose contact resistance was less than 10.0 m $\Omega$  were ranked S, samples whose contact resistance was 10.0 m $\Omega$  or more and less than 20.0 m $\Omega$  were ranked A, samples whose contact resistance was 20.0 m $\Omega$  or more and less than 50.0 m $\Omega$  were ranked B, and samples whose contact resistance was 50.0 m $\Omega$  or more were ranked C. The results are listed in Table 14.

A flowing single gas corrosion test was conducted in compliance with JIS C 5402-11-14 in the following manner to evaluate the corrosion resistance of each of the signal transfer units in the examples and comparative examples. The signal transfer unit prepared was exposed in a pollutant gas atmosphere (temperature: 30°C.; relative humidity: 75%) containing 1-ppm H<sub>2</sub>S gas on a volumetric basis. The exposure was continued for 10 days. The contact resistance of the exposed signal transfer unit was determined thereafter in the manner mentioned above. The corrosion resistance was evaluated as follows: samples whose contact resistance after the exposure was less than 10.0 m $\Omega$  were ranked S, samples whose contact resistance after the exposure was 10.0 m $\Omega$  or more and less than 20.0 m $\Omega$  were ranked A, samples whose contact resistance after the exposure was 20.0 m $\Omega$  or more and less than 50.0 m $\Omega$  were ranked B, and samples whose contact resistance after the exposure was 50.0 m $\Omega$  or more were ranked C. The results are listed in Table 14.

An abrasion loading test was conducted and contact resistance was determined in the following manner to evaluate the abrasion resistance of each of the signal transfer units in the examples and comparative examples. The contact tip of the contact probe was brought into contact with the surface of the signal transfer unit with a 100-gf pressing force using a jig, and then the contact tip of the contact probe was detached from the surface of the signal transfer unit. This operation cycle was repeated 1000 times to put an abrasion load on the surface of the signal transfer unit. The contact resistance of the loaded signal transfer unit was determined in the manner mentioned above. The abrasion resistance was evaluated as follows: samples whose contact resistance after the abrasion loading was less than 10.0 m $\Omega$  were ranked S, samples whose contact resistance after the abrasion loading was 10.0 m $\Omega$  or more and less than 20.0 m $\Omega$  were ranked A, samples whose contact resistance after the abrasion loading was 20.0 m $\Omega$  or more and less than 50.0 m $\Omega$  were ranked B, and samples whose contact resistance after the abrasion loading was 50.0 m $\Omega$  or more were ranked C. The results are listed in Table 14.

TABLE 14

| Underlayer | Coating                        |                |                         | Evaluation                   |                             |                           |
|------------|--------------------------------|----------------|-------------------------|------------------------------|-----------------------------|---------------------------|
|            | Palladium layer                |                | Pd crystalline property |                              |                             |                           |
|            | Composition/<br>Film thickness | Film thickness |                         | Gold layer<br>Film thickness | Largest<br>orientation rate | Relevant<br>crystal plane |
| Example 1  | —                              | 0.2 $\mu$ m    | 0.1%                    | —                            | 65%                         | (111)                     |
| Example 2  | —                              | 0.2 $\mu$ m    | 0.1%                    | 0.05 $\mu$ m                 | 68%                         | (111)                     |
| Example 3  | —                              | 0.2 $\mu$ m    | 0.5%                    | —                            | 71%                         | (200)                     |
| Example 4  | —                              | 0.2 $\mu$ m    | 0.5%                    | 0.05 $\mu$ m                 | 73%                         | (200)                     |
| Example 5  | —                              | 0.05 $\mu$ m   | 0.8%                    | —                            | 87%                         | (111)                     |
| Example 6  | —                              | 0.2 $\mu$ m    | 0.8%                    | —                            | 85%                         | (111)                     |

TABLE 14-continued

|                       |                      | 0.4 $\mu\text{m}$  | 0.8% | —                  | 86%       | (111) |
|-----------------------|----------------------|--------------------|------|--------------------|-----------|-------|
|                       |                      | 0.2 $\mu\text{m}$  | 0.8% | 0.05 $\mu\text{m}$ | 85%       | (111) |
|                       | Ni/4 $\mu\text{m}$   | 0.05 $\mu\text{m}$ | 0.8% | 0.05 $\mu\text{m}$ | 72%       | (200) |
| Example 10            | —                    | 0.2 $\mu\text{m}$  | 1.7% | —                  | 92%       | (200) |
| Example 11            | —                    | 0.2 $\mu\text{m}$  | 1.7% | 0.05 $\mu\text{m}$ | 80%       | (200) |
| Example 12            | —                    | 0.2 $\mu\text{m}$  | 2.5% | 0.05 $\mu\text{m}$ | 93%       | (200) |
| Example 13            | Sn/0.2 $\mu\text{m}$ | 0.2 $\mu\text{m}$  | 1.7% | —                  | 94%       | (200) |
| Example 14            | Sn/0.2 $\mu\text{m}$ | 0.2 $\mu\text{m}$  | 1.7% | 0.05 $\mu\text{m}$ | 88%       | (200) |
| Example 15            | Sn/0.2 $\mu\text{m}$ | 0.2 $\mu\text{m}$  | 2.5% | 0.05 $\mu\text{m}$ | 98%       | (200) |
| Comparative Example 1 | Ni/4 $\mu\text{m}$   | 0.2 $\mu\text{m}$  | 0.2% | —                  | 55%       | (111) |
| Comparative Example 2 | Ni/4 $\mu\text{m}$   | 0.2 $\mu\text{m}$  | 2.0% | —                  | 48%       | (200) |
| Comparative Example 3 | Ni/4 $\mu\text{m}$   | 0.2 $\mu\text{m}$  | 2.9% | —                  | Amorphous | —     |

  

| Evaluation            |                                  |            |                                  |            |                                  |            |
|-----------------------|----------------------------------|------------|----------------------------------|------------|----------------------------------|------------|
|                       | Connection reliability           |            | Corrosion resistance             |            | Abrasion resistance              |            |
|                       | Contact resistance [m $\Omega$ ] | Evaluation | Contact resistance [m $\Omega$ ] | Evaluation | Contact resistance [m $\Omega$ ] | Evaluation |
| Example 1             | 13.4                             | A          | 19.6                             | A          | 28.5                             | B          |
| Example 2             | 8.6                              | S          | 15.3                             | A          | 26.3                             | B          |
| Example 3             | 12.6                             | A          | 14.8                             | A          | 18.2                             | A          |
| Example 4             | 8.9                              | S          | 12.7                             | A          | 17.5                             | A          |
| Example 5             | 10.5                             | A          | 24.6                             | B          | 15.8                             | A          |
| Example 6             | 10.3                             | A          | 18.2                             | A          | 14.2                             | A          |
| Example 7             | 10.8                             | A          | 19.1                             | A          | 14.9                             | A          |
| Example 8             | 8.8                              | S          | 12.1                             | A          | 13.8                             | A          |
| Example 9             | 8.1                              | S          | 11.5                             | A          | 15.2                             | A          |
| Example 10            | 10.8                             | A          | 18.3                             | A          | 12.1                             | A          |
| Example 11            | 8.3                              | S          | 11.8                             | A          | 11.3                             | A          |
| Example 12            | 7.9                              | S          | 11.5                             | A          | 11.7                             | A          |
| Example 13            | 11.2                             | A          | 17.2                             | A          | 11.9                             | A          |
| Example 14            | 8.5                              | S          | 12.1                             | A          | 11.4                             | A          |
| Example 15            | 8.2                              | S          | 11.3                             | A          | 10.9                             | A          |
| Comparative Example 1 | 17.5                             | A          | 63.8                             | C          | 31.5                             | C          |
| Comparative Example 2 | 32.4                             | B          | 96.2                             | C          | 38.5                             | C          |
| Comparative Example 3 | 41.8                             | B          | 90.3                             | C          | 49.5                             | C          |

In each of the coatings in Examples 1 to 8 and 10 to 12, the palladium layer had a thickness of 0.05  $\mu\text{m}$  to 0.4  $\mu\text{m}$  and the gold layer had a thickness of 0  $\mu\text{m}$  to 0.05  $\mu\text{m}$ , in other words, they were all made thin. Such thin coatings can keep the manufacturing cost low. In addition, the coatings each including the palladium layer having a crystal plane whose orientation rate is 65% or more were proven to have sufficient corrosion resistance and connection reliability.

In each of the coatings in Examples 3 to 8 and 10 to 12, the palladium layer contained phosphorus in a concentration ranging from 0.5% by mass to 2.5% by mass, whereby the coatings were proven to have sufficient corrosion resistance, connection reliability, and abrasion resistance. In the coating in Example 9, the nickel under layer, which is less expensive, was included, whereby the coating was proven to have sufficient corrosion resistance, connection reliability, and abrasion resistance even with a thinner palladium layer.

In Examples 2, 4, 8, 9, 11, 12, 14, and 15, inclusion of the gold (Au) layer enhanced contact resistance and corrosion resistance significantly. Inclusion of the metal underlayer of Ni or Sn as the base underlying the palladium layer, i.e., in Examples 9 and 13 to 15, the whole set of evaluation values were superior to those in the comparative examples. This metal underlayer has the function of physically isolating the palladium layer from the conductor (Cu). For this purpose, besides Ni and Sn, inclusion of other metals, particularly at least one metal selected from the group consisting of Fe, Co, Zn, Rh, Ag, Pt, Au, Pb, and Bi, can still have the function of isolation. The metal underlayer can be made from an alloy containing at least one of these metal elements. The metal underlayer is made from a material different from the upper and lower layers (the palladium layer and the conductor) adjacent thereto.

It should be noted that the thickness of each layer has an acceptable error range of  $\pm 10\%$ .

## 19

The present invention can provide a coating with sufficient corrosion resistance and connection reliability and also provide an electronic component including a signal transfer unit provided with this coating thereby having sufficient corrosion resistance and connection reliability.

What is claimed is:

1. An electronic component comprising a signal transfer unit, the signal transfer unit comprising:
  - a substrate;
  - a conductor bonded to the substrate; and
  - a coating covering the conductor;
 wherein the coating comprises a palladium layer having a crystal plane whose orientation rate is 65% or more, and wherein the crystal plane whose orientation rate is 65% or more is a (111) plane or (200) plane.
2. The electronic component according to claim 1, wherein the palladium layer contains phosphorus in a concentration ranging from 0.5% by mass to 2.5% by mass.
3. The electronic component according to claim 1, further comprising a gold layer on the opposite surface of the palladium layer to the conductor.
4. The electronic component according to claim 1, further comprising a metal underlayer between the palladium layer and the conductor.
5. The electronic component according to claim 4, wherein the metal underlayer includes at least one metal selected from the group consisting of Ni, Sn, Fe, Co, Zn, Rh, Ag, Pt, Au, Pb, and Bi.
6. The electronic component according to claim 4, wherein the metal underlayer contains Ni.
7. The electronic component according to claim 3, further comprising a metal underlayer between the palladium layer and the conductor.
8. The electronic component according to claim 7, wherein the metal underlayer includes at least one metal selected from the group consisting of Ni, Sn, Fe, Co, Zn, Rh, Ag, Pt, Au, Pb, and Bi.
9. The electronic component according to claim 7, wherein the metal underlayer contains Ni.
10. The electronic component according to claim 1, wherein:
  - the conductor is copper; and
  - the palladium layer is formed by immersing the conductor in a palladium plating solution.

## 20

11. The electronic component according to claim 10, wherein a temperature of the palladium plating solution is 55° C.
12. The electronic component according to claim 10, wherein the palladium plating solution comprises:
  - diammine palladium nitrite;
  - disodium ethylenediaminetetraacetate;
  - sodium hydrogen phosphite; and
  - sodium formate.
13. The electronic component according to claim 10, wherein:
  - a surface of the conductor is activated before the conductor is immersed in the palladium plating solution; and
  - the surface of the conductor is activated by immersing the conductor in an activator liquid.
14. The electronic component according to claim 13, wherein the activator liquid comprises:
  - palladium sulfate; and
  - ammonium nitrate.
15. An electronic component comprising a signal transfer unit, the signal transfer unit comprising:
  - a substrate;
  - a conductor bonded to the substrate; and
  - a coating covering the conductor;
 wherein:
  - the coating comprises a palladium layer having a crystal plane whose orientation rate is 65% or more, wherein the crystal plane whose orientation rate is 65% or more is a (111) plane or (200) plane; and
  - the substrate is a glass epoxy substrate.
16. A signal transfer unit comprising:
  - a conductor; and
  - a coating covering the conductor;
 wherein the coating comprises a palladium layer having a crystal plane whose orientation rate is 65% or more, and wherein the crystal plane whose orientation rate is 65% or more is a (111) plane or (200) plane.
17. The signal transfer unit according to claim 16, wherein the palladium layer contains phosphorus in a concentration ranging from 0.5% by mass to 2.5% by mass.

\* \* \* \* \*